

## 1

3,415,643

HIGH TEMPERATURE FERROMAGNETIC  
COBALT-BASE ALLOY

John C. Freche, Fairview Park, Richard L. Ashbrook, Berea, Gary D. Sandrock, Cleveland, and Robert Lewis Dreshfield, Parma Heights, Ohio, assignors to the United States of America as represented by the Administrator of the National Aeronautics and Space Administration

No Drawing. Filed May 31, 1966, Ser. No. 554,950  
9 Claims. (Cl. 75—170)

The invention described herein was made by employees of the United States Government and may be manufactured and used by or for the Government for governmental purposes without the payment of any royalties thereon or therefor.

The present invention relates to improved alloys having high strength at temperatures up to 1500° F. while exhibiting high magnetic induction at low applied fields. The invention is particularly concerned with providing improved materials for use in electrical power generating equipment that is subjected to the environment of liquid metal vapor or to the vacuum of space.

Present day aerospace vehicles require space power systems having high efficiency. In order to increase the efficiency of a space power system, it is necessary to decrease the amount of power expended on cooling generators and motors. This can be accomplished by using rotor materials that have high Curie temperatures, high magnetic induction for low applied fields, and high strength at high temperatures thereby accommodating high operating temperatures.

Commercially available materials for space power system rotors include steels, such as AISI 4340, and high strength tool steel, such as H-11. Each of these steels has certain limitations. While at low temperatures, these materials have high magnetic induction for low applied fields. However, the strength of these steels falls off rapidly at about 1000° F.

One of the most desirable structural magnetic materials for use up to 1100° to 1150° F. is a cobalt-base alloy called Nivco. However, this material rapidly loses strength above 1200° F., and its magnetic induction falls off rapidly above 1300° F.

These problems have been solved by the present invention which provides a cobalt-base alloy for use as a material for rotors of electrical generators or motors to be operated at temperatures up to approximately 1400° F. These alloys can be either used as solid rotors or rolled and fabricated into laminated rotors.

It is, therefore, an object of the present invention to provide a ferromagnetic cobalt-base alloy having high strength at the elevated temperatures of liquid metal vapor in Rankine cycle turbine alternators.

Another object of the invention is to provide improved alloy materials having high Curie temperatures, high magnetic induction for low applied fields, and high strength at high temperatures, thereby permitting high operating temperatures for use in space power systems.

A still further object of the invention is to provide improved alloy materials for use in aerospace applications which are subjected to the environment of liquid metal vapor or to the hard vacuum of space.

These and other objects and advantages of the inven-

## 2

tion will be apparent from the specification which follows.

The present invention is embodied in alloys having the following nominal composition range:

5 Cobalt ----- From about 71.5 percent to about 94.3  
Tungsten ----- From about 5 percent to about 14  
Titanium ----- From about 0.3 percent to about 1.8  
Zirconium ----- From about 0.1 percent to about 1.0  
Carbon ----- From about 0.3 percent to about 0.7  
Iron ----- From about 0 percent to about 10

10 A preferred embodiment of the invention includes alloys having the following nominal composition range:

Cobalt ----- From 82.9 percent to 87.9  
15 Tungsten ----- From 7.5 percent to 10  
Titanium ----- 1  
Zirconium ----- 0.5  
Carbon ----- 0.6  
Iron ----- From 2.5 percent to 5

20 An alloy composition used where high strength is of paramount importance has the following nominal composition:

|           | Percent |
|-----------|---------|
| 25 Cobalt | 85.9    |
| Tungsten  | 12.0    |
| Titanium  | 1.0     |
| Zirconium | 0.5     |
| Carbon    | 0.6     |

30 The subject alloys were prepared by vacuum induction melting. However, it is contemplated that these alloys can also be prepared by induction melting under a protective atmosphere of argon.

35 The subject alloys were prepared in a vacuum induction melting furnace capable of reaching pressures as low as  $10^{-4}$  torr. and holding pressures as low as  $5 \times 10^{-3}$  torr. during active boiling of the melt. Raw materials were charged both into a zirconia crucible as well as into an "addition's-maker." After the crucible charge was melted, the melt was refined by permitting the oxygen in the charge to react with carbon to produce a so-called "carbon boil." After refining, the portion of the charge containing the reactive elements, titanium and zirconium, was added to the melt which was then heated to an appropriate casting temperature. The melt was then poured into ceramic shell molds heated to 1600° F.

40 Although vacuum induction melting was used in the development of this alloy series, similar alloys have been successfully induction melted under an argon atmosphere. These alloys are likewise amenable to melting by the electro-slag process where protection from the atmosphere is partially provided by a layer of slag rather than solely by vacuum or an inert gas.

45 The above listed alloys derive their high elevated temperature strength from the solid solution strengthening of cobalt by tungsten, by the precipitation of an intermediate phase of  $WCo_3$ , and by the presence of dispersed tungsten, titanium and zirconium carbides. The good magnetic and strength properties are the result of a compromise between the tungsten and iron content in the alloy. The iron contributes to the high induction and structural stability while the tungsten contributes to the high strength.

50 Various magnetic and mechanical properties of the preferred composition compared with those of one of the

strongest cobalt-base high temperature magnetic alloys commercially available are shown in Table I.

applied fields at elevated temperatures consisting essentially of from 5% to 14% tungsten, from .3% to 1.8%

TABLE I.—MAGNETIC AND MECHANICAL PROPERTIES OF SELECTED ALLOYS

| Property                                                      | Test tempera-<br>ture, ° F. | Alloy              |         |                    |                     |
|---------------------------------------------------------------|-----------------------------|--------------------|---------|--------------------|---------------------|
|                                                               |                             | 7.5W-2.5Fe         | 10W-5Fe | 12 W               | Nivco               |
| Ultimate tensile strength, p.s.i.                             | 1,300                       | 57,200             | 58,000  | 59,000             | <sup>1</sup> 95,000 |
|                                                               | 1,400                       | 46,350             | 48,000  | 52,600             | 49,500              |
|                                                               | 1,500                       | 41,000             | 49,000  | 50,000             | <sup>2</sup> 29,000 |
|                                                               | 1,600                       | —                  | —       | —                  | 22,000              |
| Stress rupture life at stress of 45,000 p.s.i. in hours.      | 1,700                       | 33,600             | 32,200  | 35,500             | —                   |
|                                                               | 1,200                       | <sup>2</sup> 50    | 90      | <sup>1</sup> 1,268 | 750                 |
|                                                               | 1,300                       | 25                 | 433     | 1,290              | 30                  |
|                                                               | 1,400                       | 1.2                | 96      | 392                | 1                   |
| Magnetic induction in kilogausses for field of 100<br>gausses | 1,400                       | 10.3               | 9.2     | 8.2                | 9.4                 |
| Curie temperature, ° F.                                       | —                           | <sup>2</sup> 1,820 | 1,710   | 1,690              | 1,690               |

<sup>1</sup> Stress 50,000 p.s.i.  
<sup>2</sup> Extrapolated.  
<sup>3</sup> Interpolated.

There are other alloys suitable for magnetic applications at elevated temperatures. Among these are H-11 and 18% nickel-maraging steel. However, their use is limited to temperatures below 1000° F. because of microstructural instabilities. The lowest test temperature shown in Table I is 1200° F.

It has also been found that the stress rupture properties of the alloy series can be improved by heat treating. Two such heat treatments have been found to improve the stress rupture properties of the alloy Co-7.5W-2.5Fe-1Ti-0.5Zr-0.6C in the range from 1200° to 1400° F. According to the invention, the alloy was heated for 72 hours at either 1700° F. or 1500° F. Table II illustrates the effect of such heat treatments on mechanical properties of the alloy as compared to Nivco 10.

TABLE II.—EFFECT OF HEAT TREATMENT ON MECHANICAL PROPERTIES OF SELECTED ALLOY

| Property                                               | Test tempera-<br>ture, ° F. | Alloy                        |                                   |           |
|--------------------------------------------------------|-----------------------------|------------------------------|-----------------------------------|-----------|
|                                                        |                             | Co-7.5W-2.5Fe-1Ti-0.5Zr-0.6C |                                   |           |
|                                                        |                             | As-cast                      | Heat-treated—aging<br>temperature | Nivco     |
| Average ultimate tensile strength (p.s.i.)             | 1,200                       | 55,800                       | 1,700° F.                         | 1,500° F. |
|                                                        | 1,300                       | 57,200                       | 53,400                            | 53,300    |
|                                                        | 1,400                       | 46,350                       | 51,500                            | 51,100    |
|                                                        | 1,500                       | 41,100                       | 46,000                            | 46,400    |
| Average stress rupture life at 45,000 p.s.i. in hours. | 1,200                       | <sup>1</sup> 50              | 42,300                            | 29,000    |
|                                                        | 1,300                       | 25                           | 2,500                             | —         |
| Average stress rupture life at 40,000 p.s.i. in hours. | 1,400                       | 25                           | 400                               | 1,700     |
|                                                        | 1,400                       | —                            | 30                                | 30        |
| Magnetic induction in kilogausses                      | 1,400                       | 10.3                         | 10.3                              | 300       |

<sup>1</sup> Extrapolated.

The beneficial technical effect of heat treatment on stress rupture properties is associated with the formation of a finely dispersed precipitate in the material. The aging treatments do not significantly affect the tensile strength. Depending on the test conditions, both slight increases and slight decreases in tensile strength have been observed. However, the greatest room temperature ductility was obtained after aging at 1700° F. for 72 hours. Both heat treatments resulted in improved properties over the as cast condition and over the commercial alloy Nivco 10.

The examples set forth above describe the properties of castings made in accordance with the invention. It is contemplated that the cast alloys will be worked into sheet material by forging or rolling for use in making laminated structures, such as rotors, when it is desired to minimize eddy current losses. Conventional hot rolling techniques have been used to obtain sheet material for these alloys. A satisfactory annealing treatment for the sheet has been found to be one-half hour at 2350° F.

It is understood that equivalents or modifications of or substitutions for parts of the above-described embodiments of the invention may be made without departing from the spirit of the invention or the scope of the subjoined claims.

What is claimed is:

1. A cobalt base alloy having a high Curie temperature, high strength and high magnetic induction for low

titanium, from 0.1% to 1% zirconium, from 0.3% to 0.7% carbon, up to 10% iron, and the rest essentially cobalt.

2. A cobalt base alloy having a high Curie temperature, high strength and high magnetic induction for low applied fields at elevated temperatures consisting essentially of 1.0% titanium, 0.5% zirconium, 0.6% carbon, from 7.5% to 10% tungsten, 2.5% to 5% iron, and the rest cobalt.

3. A cobalt base alloy as claimed in claim 2 containing 7.5% tungsten, 2.5% iron and about 87.9% cobalt.

4. A cobalt base alloy as claimed in claim 2 including 10% tungsten, 5% iron, and about 82.9% cobalt.

5. A cobalt base alloy as claimed in claim 2 including 10% tungsten, 2.5% iron, and about 85.4% cobalt.

6. A cobalt base alloy consisting essentially of 12% tungsten, 1.0% titanium, 0.5% zirconium, 0.6% carbon, and about 85.9% cobalt.

50 7. A method of making a high strength ferromagnetic material having improved electrical properties at temperatures up to 1400° F. comprising the steps of casting an alloy having a composition essentially in the range of about 5% to 14% tungsten, .3% to 1.8% titanium, 0.1% to 1% zirconium, 0.3% to 0.7% carbon, up to 10% iron, and the rest cobalt, and heat treating the alloy to improve the strength thereof by aging for about 72 hours at a temperature in the range from about 1300° F. to about 1700° F.

60 8. A method of making a high strength ferromagnetic material as claimed in claim 7 including the step of working the cast alloy into sheet.

9. A method of making a high strength ferromagnetic material as claimed in claim 8 including the step of annealing the sheet at 2350° F. for one-half hour.

#### References Cited

#### UNITED STATES PATENTS

3,271,140 9/1966 Freche et al. ----- 75—170  
70 3,276,865 10/1966 Freche et al. ----- 75—170

RICHARD O. DEAN, Primary Examiner.

U.S. CL. X.R.

75 148—158, 12.7, 31.55, 2, 3, 32.5